# EUROPEAN PATENT SPECIFICATION

(11) **EP 2 208 547 B1**
(45) Date of publication and mention of the grant of the patent: **30.07.2014**
(21) Application number: 08839763.3
(22) Date of filing: 15.10.2008
(51) Int. Cl.: B21B 3/00, B21B 1/26

(54) **MAGNESIUM HOT ROLLING METHOD AND APPARATUS**
VERFAHREN UND VORRICHTUNG ZUM WARMWALZEN VON MAGNESIUM
PROCÉDÉ ET APPAREIL DE LAMINAGE À CHAUD DE MAGNÉSIUM

(30) Priority: 16.10.2007 JP 2007269058
(43) Date of publication of application: 21.07.2010
(73) Proprietor: IHI Corporation, Tokyo 135-8710 (JP)
(72) Inventor: TAZOE, Nobuhiro, Tokyo 105-0004 (JP); HONJOU, Hisashi, Yokohama-shi Kanagawa 235-8501 (JP); MATSUMURA, Hideo, Yokohama-shi Kanagawa 235-8501 (JP); YANAI, Katuhiko, Hitachiomiya-shi Ibaraki 319-2134 (JP); YANAI, Fumitaka, Hitachiomiya-shi Ibaraki 3192134 (JP)
(74) Representative: Lamb, Martin John Carstairs
(86) International application number: PCT/JP2008/068654
(87) International publication number: WO 2009/051134

(56) References cited:
- WO-A1-03/008121
- JP-A- 05 015 905
- JP-A- 08 010 805
- JP-A- 08 264 261
- JP-A- 63 220 901
- JP-A- 2003 112 205
- JP-A- 2004 066 302
- JP-A- 2004 090 065
- JP-B2- 3 119 692
- JP-B2- 05 045 327
- US-A1- 2004 079 513

## Description

### [Technical Field]

The present invention relates to a magnesium hot rolling method and to a magnesium hot rolling apparatus.

### [Technical Background]

To manufacture a magnesium sheet from magnesium alloy, a round bar-shaped billet having, for example, a diameter of approximately 300 to 400 mm and a length of approximately 500 to 600 mm is molded by hot extrusion molding into a thick plate having a thickness of, for example, 10 mm or less. This thick plate is then cut to a predetermined length (for example, 3 m) so as to form a cut plate material, and this cut plate material is then rolled to a thickness of not more than1 mm by rough rolling.

In order to roll magnesium alloy at room temperature a large amount of pressure is required. However, even if a large amount of pressure is applied, it still cracks easily. Accordingly, it is preferably rolled using hot rolling.

Conventional examples of apparatuses for the hot rolling of magnesium alloy are disclosed in FIG. 1 of patent document 1 and FIG. 1 of patent document 2.

The hot rolling apparatuses disclosed in these patent documents are provided with a rolling mill which rolls the magnesium alloy while transporting it reciprocatingly, and with two heating furnaces which are located on the upstream side and the downstream side of the rolling mill. The magnesium alloy is heated to a predetermined temperature by these heating furnaces and is rolled in the rolling mill.
[Patent document 1] Japanese Patent Publication No. 3521863
[Patent document 2] Japanese Patent Publication No. 3821074
Reference is also made to JP2004-066302, which discloses a magnesium hot rolling method and apparatus according to the preambles of claims 1 and 3 respectively.

### [Disclosure of the Invention]

### [Problems to be Solved by the Invention]

However, in the hot rolling apparatuses disclosed in the aforementioned patent documents, because heating furnaces are only provided on both sides of the rolling mill, as the magnesium cut plate material becomes gradually elongated by the reciprocating rolling, the ends of the magnesium cut plate material begin to protrude from the heating furnaces and these protruding portions cool down. The reason why this is a problem is because temperature variations in the magnesium cut plate material during the hot rolling cause errors in the dimensional accuracy and a deterioration in the quality of a finished product.

The present invention was conceived in view of the above described circumstances and it is an object thereof to provide a magnesium hot rolling method and a magnesium hot rolling apparatus which are able to prevent any reduction in the quality of a product which is due to temperature variations during the hot rolling of a magnesium alloy.

### [Means for Solving the Problem]

In order to solve the above described problems, the following apparatuses and methods are employed in the present invention.

As a first aspect of the present invention, a magnesium alloy hot rolling method is employed which has: a first rolling step in which a magnesium plate is rolled reciprocatingly between an upstream heating furnace which is located on an upstream side of a rolling mill and which heats the magnesium plate, and a downstream heating furnace which is located on a downstream side of the rolling mill and which heats the magnesium plate; and a second rolling step in which the temperature of respective end portions of the magnesium plate on both the upstream and downstream sides is maintained while the magnesium plate is being rolled reciprocatingly between an upstream temperature maintaining apparatus which is located further on the upstream side than the upstream heating furnace and which transports the magnesium plate which has been heated by the upstream heating furnace while maintaining the temperature thereof, and a downstream temperature maintaining apparatus which is located further on the downstream side than the downstream heating furnace and which transports the magnesium plate which has been heated by the downstream heating furnace while maintaining the temperature thereof.

In the magnesium alloy hot rolling method according to the above described first aspect of the present invention, it is also possible for there to be provided a wind-on step in which, while tension is applied by a tension applying apparatus which is located on the downstream side of the downstream temperature maintaining apparatus to the magnesium plate which has been rolled to a predetermined thickness, the magnesium plate is wound onto a winder which is placed further on the downstream side than the downstream temperature maintaining apparatus.

As a second aspect of the present invention, a magnesium alloy hot rolling apparatus is employed which is provided with: a rolling mill which performs reciprocating rolling on a magnesium plate; an upstream heating furnace which is located on the upstream side of the rolling mill and which heats the magnesium plate; a downstream heating furnace which is located on the downstream side of the rolling mill and which heats the magnesium plate; an upstream temperature maintaining apparatus which is located further on the upstream side than the upstream heating furnace, and which transports the magnesium plate which has been heated by the upstream heating furnace and also maintains the temperature of upstream side end portions thereof; and a downstream temperature maintaining apparatus which is located further on the downstream side than the downstream heating furnace, and which transports the magnesium plate which has been heated by the downstream heating furnace and also maintains the temperature of downstream side end portions thereof.

In the magnesium alloy hot rolling apparatus according to the above described second aspect of the present invention, it is also possible for a plurality of groups of pinch rollers which sandwich the magnesium plate in the thickness direction thereof and adjust the transporting speed thereof to be provided respectively between the rolling mill and the upstream heating furnace and between the rolling mill and the downstream heating furnace.

In the magnesium alloy hot rolling apparatus according to the above described second aspects of the present invention, it is also possible for working rollers of the rolling mill and the plurality of groups of pinch rollers which are located on the upstream and downstream sides of the rolling mill to be heating rollers.

In the magnesium alloy hot rolling apparatus according to the above described second aspects of the present invention, it is also possible for there to be provided: a tension applying apparatus which is located on the downstream side of the downstream temperature maintaining apparatus and which applies tension to the magnesium plate; and a winder which is located further on the downstream side than the tension applying apparatus and onto which the magnesium plate is wound.

### [Effects of the Invention]

According to the present invention, because a magnesium plate is rolled while substantially the entire length thereof is being heated and held at a predetermined temperature, it is possible to suppress any drop in the temperature of the magnesium plate, and to prevent errors in the dimensional accuracy of a product as well as any consequent deterioration in product quality which are due to temperature variations during hot rolling, and to thus maintain a superior quality in a finished product.

### [Brief description of the drawings]

[FIG. 1] FIG. 1 is a schematic front view showing the schematic structure of a hot rolling apparatus in an embodiment of the present invention.
[FIG. 2] FIG. 2 is a typical view showing the schematic structure of a leveler.

### [Description of the Reference Numerals]

- 100: Hot rolling apparatus (magnesium hot rolling apparatus)
- 1: Rolling mill
- 2: First heating furnace (upstream heating furnace)
- 3: Second heating furnace (downstream heating furnace)
- 4: Pinch roller (feed roller pair)
- 5: First table roller (upstream temperature maintaining apparatus)
- 6: Second table roller (downstream temperature maintaining apparatus)
- 7: Winder
- 8: Pinch rollers (tension applying apparatus)
- M0: Magnesium cut plate material (magnesium plate)
- M1: Magnesium sheet (magnesium plate)

### [Best Embodiments for Implementing the Invention]

An embodiment of the present invention will now be described with reference made to the drawings.

FIG. 1 is a schematic front view showing the schematic structure of a hot rolling apparatus 100 (i.e., a magnesium alloy hot rolling apparatus) in the present embodiment.

As is shown in FIG. 1, the hot rolling apparatus 100 according to the present embodiment is provided with a rolling mill 1, a first heating furnace 2, a second heating furnace 3, pinch rollers 4, a first table roller 5, a second table roller 6, a winder 7, and pinch rollers 8.

The rolling mill 1 has a pair of working rollers 1a that are in parallel with each other and also face each other, and with a drive source (not shown) which drives the working rollers I a to rotate.

The working rollers 1a are heating rollers whose surface temperature is raised to a suitable temperature and which, while feeding a magnesium cut plate material M0 (i.e., a magnesium plate) which is passing between the working rollers 1a in one direction, apply predetermined pressure to this magnesium cut plate material M0. As a result of this, the rolling mill 1 reduces the thickness of the magnesium cut plate material M0 so as to cause it to become elongated.

Moreover, the rolling mill 1 performs reciprocating rolling by reversing the feed direction of the magnesium cut plate material M0 at a predetermined timing. By doing this, the rolling mill 1 reduces the thickness of the magnesium cut plate material M0 from, for example, a thickness of approximately 6 mm and a length of approximately 3 m to a thickness of approximately 1 mm and a length of approximately 18 m.

Note that the above described magnesium cut plate material M0 (i.e., magnesium plate) which forms a work piece for this hot rolling apparatus 100 is a plate material formed from magnesium alloy

The first heating furnace 2 (i.e., the upstream heating furnace) is a heating furnace which is located on the upstream side of the rolling mill 1. The second heating furnace 3 (i.e., the downstream heating furnace) is a heating furnace which is located on the downstream side of the rolling mill 1.

The pair of heating furnaces 2 and 3 have a length which is longer than that of the magnesium cut plate material M0 prior to rolling, and are also provided with heaters and transporting rollers (neither are shown). The magnesium cut plate material M0 is heated by the heaters to a predetermined temperature (approximately 100 to 350 °C with 200 to 300 °C being preferable), and the magnesium cut plate material M0 is transported by the transporting rollers.

The pinch rollers 4 are heating rollers whose surface temperature is raised to a suitable temperature, and they provide auxiliary transporting for the magnesium cut plate material M0 which is traveling reciprocatingly in conjunction with the reciprocating rolling of the rolling mill 1. A plurality of sets of these pinch rollers 4 are provided respectively between the rolling mill 1 and the first heating furnace 2, and between the rolling mill 1 and the second heating furnace 3.

By adjusting the transporting speed, the pinch rollers 4 can be made to apply suitable tension to the magnesium cut plate material M0 which is being rolled by the rolling mill 1.

The first table roller 5 (i.e., the upstream temperature maintaining apparatus) is located on the upstream side of the first heating furnace 2, while the second table roller 6 (i.e., the downstream temperature maintaining apparatus) is located on the downstream side of the second heating furnace 3. These table rollers 5 and 6 each have transporting rollers 5a and 6a and temperature maintaining covers 5b and 6b.

When the magnesium cut plate material M0 becomes elongated by being reverse rolled by the rolling mill 1, the end portions thereof protrude from the heating furnaces 2 and 3. The table rollers 5 and 6 transport and support the end portions of the magnesium cut plate material M0 which are protruding from the heating furnaces 2 and 3 using the transporting rollers 5a and 6a, and also shield them from the outside air by covering them with the temperature maintaining covers 5b and 6b. As a result, the table rollers 5 and 6 maintain the temperature of the magnesium cut plate material M0 by not allowing heat to escape therefrom. Moreover, during reverse rolling the temperature maintaining portion of the end portion of the magnesium cut plate material M0 which is positioned on the downstream side is moved inside the heating furnace during the subsequent rolling in the opposite direction. In addition, the heating portion of the end portion which is positioned on the downstream side is placed inside the temperature maintaining apparatus during the rolling in the opposite direction, and by repeating this process alternatingly, it is possible to minimize any reduction in the temperature of the end portions.

The winder 7 is a machine onto which is wound the manufactured product obtained by rolling the magnesium cut plate material M0, namely, a magnesium sheet M1 (i.e., a magnesium plate).

The pinch rollers 8 (i.e., the tension applying apparatus) are located in front of the winder 7 and by adjusting the transporting speed of the magnesium sheet M1, they are able to apply tension to the magnesium sheet M1 in the opposite direction from the wind-on direction of the winder 7.

Using this type of structure, the hot rolling apparatus 100 performs rough rolling on the magnesium cut plate material M0. Hereinafter, an operation of the hot rolling apparatus 100 will be described.

Firstly, the magnesium cut plate materials M0 which are the objects to be rolled by this hot rolling apparatus 100 are manufactured by performing hot extrusion molding (at between approximately 100 and 300 °C with 200 °C being preferable) on a rod-shaped billet having, for example, a diameter of 300 to 400 mm and a length of 500 to 600 mm so as to mold it into a thick plate having a thickness of, for example, 10 mm or less (for example, 6 mm). This thick plate is then cut into predetermined lengths (for example, 3 m).

Because the crystal grains of the magnesium forming the magnesium cut plates M0 which have been molded by hot extrusion molding are mechanically refined by being extruded, they are extremely strong and are of high quality. They are also difficult to break and have superior press-moldability.

The magnesium cut plate materials M0 are transported from the first table rollers 5 to the first heating furnace 2. They are then heated to a predetermined temperature (approximately 100 to 350 °C with 200 to 300 °C being preferable) inside the first heating furnace 2 and are then transported to the rolling mill 1.

The rolling mill 1 rolls the magnesium cut plate material M0 and, at the same time as this, transports it to the second heating furnace 3. The temperature of the magnesium cut plate materials M0 drops somewhat as it moves from the first heating furnace 2 to the second heating furnace 3. However, because the working rollers 1a and the plurality of pinch rollers 4 are heating rollers, and because the magnesium cut plate material M0 is once again heated to the predetermined temperature inside the second heating furnace 3, there is little temperature variation.

When the terminal end of a magnesium cut plate material M0 has passed through the rolling mill 1, the hot rolling apparatus 100 reverses the rolling direction. The hot rolling apparatus 100 repeats this process so that the magnesium cut plate material M0 is rolled reciprocatingly, and the thickness of the magnesium cut plate material M0 is sequentially reduced. As a result, a magnesium sheet M1 is manufactured.

Here, specific examples of the respective numerical values for the rough rolling performed by this hot rolling apparatus 100 are shown below in Table 1.

**[Table 1]**

| Pass No. | Entry side thickness (mm) | Reduction amount (mm) | Rolling temperature (°C) | Rolling speed (m/min) | Rolling load (ton) |
|---|---|---|---|---|---|
| 1 | 6.00 | 1.80 | 200 | 10 | 180 |
| 2 | 4.20 | 1.26 | 200 | 10 | 165 |
| 3 | 2.94 | 0.88 | 200 | 10 | 150 |
| 4 | 2.06 | 0.62 | 200 | 10 | 140 |
| 5 | 1.44 | 0.43 | 200 | 10 | 135 |

| | | | | | |
|---|---|---|---|---|---|
| Final thickness 1.01 mm | | | | | |

In the above specific examples, the magnesium cut plate material M0 has a material quality of AZ31B, and has dimensions of a thickness of 6.00 mm, a width of 300 mm, and a length of 3000 mm. The diameter of the working rollers 1a is 400 mm and the barrel length thereof is 500 mm, while the diameter of the pinch rollers 4 is 250 mm.

Moreover, in the above described examples, the heating temperature in the heating furnaces 2 and 3 is 220 °C, while the pinch rollers 4 and the working rollers 1 a are heating rollers having internal heaters and the surface temperature of these heating rollers is 200 °C.

In addition, in the above example, a magnesium cut plate material M0 having a thickness of 6.00 mm is changed by five passes of reciprocating rolling (i.e., by two and a half reciprocations) into a magnesium sheet M1 having a thickness of 1.01 mm, and this is then wound onto the winder 7 after the five passes.

The magnesium cut plate material M0 becomes gradually more elongated as it is rolled, and when the terminal end thereof has passed through the rolling mill 1, the end portions including the starting end protrude from the heating furnaces 2 and 3.

The table rollers 5 and 6 support the end portions which are protruding from the heating furnaces 2 and 3 using the transporting rollers 5a and 6a, and also maintain the temperature thereof by means of the temperature maintaining covers 5b and 6b.

This will now be described in more detail using FIG. 1. For example, a magnesium cut plate material M0 having a length L0 prior to rolling is rolled in a section A1 until it attains a length L1 (first rolling step). It is then rolled in a section A2 until it exceeds the length L1 and attains a length L2 (second rolling step). It is then wound on (winding-on step).

Thus, this hot rolling apparatus 100 performs reciprocating rolling using the first rolling step in the section A1, namely, in the section formed by the first heating furnace 2, the rolling mill 1, and the second heating furnace 3 while the magnesium cut plate material M0 has a length between L0 and L1. The hot rolling apparatus 100 then performs reciprocating rolling using the second rolling step in the section A2, that is, in the section formed by the first table roller 5, the first heating furnace 2, the rolling mill 1, the second heating furnace 3, and the second table roller 6 after the magnesium cut plate material M0 has exceeded the length L1 and until it attains the length L2. The finished product, namely, the magnesium sheet M1 is then wound onto the winder 7.

As a result, the magnesium cut plate M0 is heated or has its temperature maintained over its entire length, and is kept at a temperature which remains substantially within a fixed range. Accordingly, it is possible to prevent any reduction in the quality of a product which is due to temperature variations in the magnesium cut plate material M0, and it is possible to maintain a superior quality in the finished product, namely, in the magnesium sheet M1.

The magnesium cut plate material M0 is soft during the rolling process due to the high temperature, and there is a possibility that pitting will remain if high pressure is also applied to areas other than those areas where the rolling mill 1 is used. However, in contrast to this, in this hot rolling apparatus 100, because the magnesium cut plate material M0 is nipped in a plurality of locations by a plurality of groups of pinch rollers 4, the force with which each pinch roller 4 nips the magnesium cut plate material M0 is small as a result of being dispersed, and any concern that pitting from the pinch rollers 4 will remain is reduced.

In addition, once the thickness of the magnesium cut plate material M0 has been rolled down to a predetermined thickness (for example, 1 mm) so as to form the magnesium sheet M1, the hot rolling apparatus 100 winds this magnesium sheet M1 onto the winder 7 so as to form a coil material.

At this time, the pinch rollers 8 adjust the transporting speed of the magnesium sheet M1 so that predetermined tension is applied to the magnesium sheet M1 being wound onto the winder 7, and thereby apply tensile force to the magnesium sheet M1 in the opposite direction from the wind-on direction of the winder 7.

According to the hot rolling apparatus 100 of the present invention, because the magnesium cut plate material M0 is rolled while substantially the entire length thereof is being heated and held at a predetermined temperature, it is possible to suppress any drop in the temperature of the magnesium cut plate material M0, and to prevent any reduction in the product quality which is due to temperature variations during the hot rolling, and it is thereby possible to maintain a superior quality in the finished product, namely, in the magnesium sheet M1.

Note that in the present embodiment, the pinch rollers 8 function as a tension applying apparatus, however, the tension applying apparatus may also be formed by a leveler which flattens the magnesium sheet M1.

Here, as is shown in FIG. 2, the leveler is formed by alternatingly combining three or more rollers in two rows in a beehive pattern when viewed in cross-section, and the magnesium sheet M1 is flattened as a result of the sheet-shaped material being passed between these rollers.

### [Industrial applicability]

According to the magnesium hot rolling apparatus of the present invention and to the magnesium hot rolling method of the present invention which uses this apparatus, it is possible to prevent errors in the dimensional accuracy of a product as well as any consequent deterioration in product quality which are due to temperature variations during hot rolling, and to also maintain a superior quality in a finished product.

## Claims

1. A magnesium alloy hot rolling method comprising:
a first rolling step in which a magnesium plate (M1) is rolled reciprocatingly between an upstream heating furnace (2) which is located on an upstream side of a rolling mill (1) and which heats the magnesium plate, and a downstream heating furnace (3) which is located on a downstream side of the rolling mill (1) and which heats the magnesium plate (M1); **characterized by** further comprising:
a second rolling step in which the temperature of respective end portions of the magnesium plate (M1) on both the upstream and downstream sides is maintained while the magnesium plate (M1) is being rolled reciprocatingly between an upstream temperature maintaining apparatus (5) which is located further on the upstream side than the upstream heating furnace (2) and which transports the magnesium plate (M1) which has been heated by the upstream heating furnace (2) while maintaining the temperature thereof, and a downstream temperature maintaining apparatus (6) which is located further on the downstream side than the downstream heating furnace (3) and which transports the magnesium plate (M1) which has been heated by the downstream heating furnace (3) while maintaining the temperature thereof.

2. The magnesium alloy hot rolling method according to claim 1, wherein there is provided a wind-on step in which, while tension is applied by a tension applying apparatus (8) which is located on the downstream side of the downstream temperature maintaining apparatus (6) to the magnesium plate (M1) which has been rolled to a predetermined thickness, the magnesium plate (M1) is wound onto a winder (7) which is placed further on the downstream side than the downstream temperature maintaining apparatus (6).

3. A magnesium alloy hot rolling apparatus comprising:
a rolling mill (1) which performs reciprocating rolling on a magnesium plate (M1);
an upstream heating furnace (2) which is located on the upstream side of the rolling mill (1) and which heats the magnesium plate (M1); and
a downstream heating furnace (3) which is located on the downstream side of the rolling mill (1) and which heats the magnesium plate (M1);
**characterized in that** the apparatus further comprises:
an upstream temperature maintaining apparatus (5) which is located further on the upstream side than the upstream heating furnace (2), and which transports the magnesium plate (M1) which has been heated by the upstream heating furnace (2) and also maintains the temperature of upstream side end portions thereof; and
a downstream temperature maintaining apparatus (6) which is located further on the downstream side than the downstream heating furnace(3), and which transports the magnesium plate (M1) which has been heated by the downstream heating furnace (3) and also maintains the temperature of downstream side end portions thereof.

4. The magnesium alloy hot rolling apparatus according to claim 3, wherein a plurality of groups of pinch rollers (4) which sandwich the magnesium plate (M1) in the thickness direction thereof and adjust the transporting speed thereof are provided respectively between the rolling mill (1) and the upstream heating furnace (2) and between the rolling mill (1) and the downstream heating furnace (3).

5. The magnesium alloy hot rolling apparatus according to claim 4, wherein working rollers of the rolling mill (1) and the plurality of groups of pinch rollers (4) which are located on the upstream and downstream sides of the rolling mill (1) are heating rollers.

6. The magnesium hot rolling apparatus according to claim 3 or 4, wherein there are provided:
a tension applying apparatus (8) which is located on the downstream side of the downstream temperature maintaining apparatus (6) and which applies tension to the magnesium plate (M1); and
a winder (7) which is located further on the downstream side than the tension applying apparatus (8) and onto which the magnesium plate (M1) is wound.

## Patentansprüche

1. Magnesiumlegierung-Warmwalzverfahren, das Folgendes umfasst:
einen ersten Walzschritt, in dem eine Magnesiumplatte (M1) hin- und hergehend zwischen einem stromaufwärts gelegenen Wärmeofen (2), der auf einer stromaufwärts gelegenen Seite eines Walzwerks (1) angeordnet ist und der die Magnesiumplatte erwärmt, und einem stromabwärts gelegenen Wärmeofen (3), der auf einer stromabwärts gelegenen Seite des Walzwerks (1) angeordnet ist und der die Magnesiumplatte (M1) erwärmt, gewalzt wird, **dadurch gekennzeichnet, dass** es ferner Folgendes umfasst:
einen zweiten Walzschritt, in dem die Temperatur jeweiliger Endabschnitte der Magnesiumplatte (M1) sowohl auf der stromaufwärts als auch auf der stromabwärts gelegenen Seite aufrechterhalten wird, während die Magnesiumplatte (M1) hin- und hergehend zwischen einer stromaufwärts gelegenen Temperaturerhaltungsvorrichtung (5), die weiter auf der stromaufwärts gelegenen Seite angeordnet ist als der stromaufwärts gelegene Wärmeofen (2) und welche die Magnesiumplatte (M1), die durch den stromaufwärts gelegenen Wärmeofen (2) erwärmt worden ist, befördert, während sie die Temperatur derselben aufrechterhält, und einer stromabwärts gelegenen Temperaturerhaltungsvorrichtung (6), die weiter auf der stromabwärts gelegenen Seite angeordnet ist als der stromabwärts gelegene Wärmeofen (3) und welche die Magnesiumplatte (M1), die durch den stromabwärts gelegenen Wärmeofen (3) erwärmt worden ist, befördert, während sie die Temperatur derselben aufrechterhält, gewalzt wird.

2. Magnesiumlegierung-Warmwalzverfahren nach Anspruch 1, wobei ein Aufwickelschritt bereitgestellt wird, bei dem, während durch eine Spannungsausübungsvorrichtung (8), die auf der stromabwärts gelegenen Seite der stromabwärts gelegenen Temperaturerhaltungsvorrichtung (6) angeordnet ist, Spannung auf die Magnesiumplatte (M1), die auf eine vorbestimmte Dicke gewalzt worden ist, ausgeübt wird, die Magnesiumplatte (M1) auf eine Aufwickelvorrichtung (7) gewickelt wird, die weiter auf der stromabwärts gelegenen Seite angeordnet ist als die stromabwärts gelegene Temperaturerhaltungsvorrichtung (6).

3. Magnesiumlegierung-Warmwalzvorrichtung, die Folgendes umfasst:
ein Walzwerk (1), das ein hin- und hergehendes Walzen an einer Magnesiumplatte (M1) ausführt,
einen stromaufwärts gelegenen Wärmeofen (2), der auf der stromaufwärts gelegenen Seite des Walzwerks (1) angeordnet ist und der die Magnesiumplatte (M1) erwärmt, und
einen stromabwärts gelegenen Wärmeofen (3), der auf einer stromabwärts gelegenen Seite des Walzwerks (1) angeordnet ist und der die Magnesiumplatte (M1) erwärmt,
**dadurch gekennzeichnet, dass** die Vorrichtung ferner Folgendes umfasst:
eine stromaufwärts gelegene Temperaturerhaltungsvorrichtung (5), die weiter auf der stromaufwärts gelegenen Seite angeordnet ist als der stromaufwärts gelegene Wärmeofen (2) und welche die Magnesiumplatte (M1), die durch den stromaufwärts gelegenen Wärmeofen (2) erwärmt worden ist, befördert und die ebenfalls die Temperatur von stromaufwärtsseitigen Endabschnitten derselben aufrechterhält, und
eine stromabwärts gelegene Temperaturerhaltungsvorrichtung (6), die weiter auf der stromabwärts gelegenen Seite angeordnet ist als der stromabwärts gelegene Wärmeofen (3) und welche die Magnesiumplatte (M1), die durch den stromabwärts gelegenen Wärmeofen (3) erwärmt worden ist, befördert und die ebenfalls die Temperatur von stromabwärtsseitigen Endabschnitten derselben aufrechterhält.

4. Magnesiumlegierung-Warmwalzvorrichtung nach Anspruch 3, wobei mehrere Gruppen von Klemmwalzen (4), welche die Magnesiumplatte (M1) in der Dickenrichtung derselben einklemmen und die Beförderungsgeschwindigkeit derselben einstellen, jeweils zwischen dem Walzwerk (1) und dem stromaufwärts gelegenen Wärmeofen (2) beziehungsweise zwischen dem Walzwerk (1) und dem stromabwärts gelegenen Wärmeofen (3) bereitgestellt werden.

5. Magnesiumlegierung-Warmwalzvorrichtung nach Anspruch 4, wobei Arbeitswalzen des Walzwerks (1) und die mehreren Gruppen von Klemmwalzen (4), die auf der stromaufwärts und der stromabwärts gelegenen Seite des Walzwerks (1) angeordnet sind, Wärmewalzen sind.

6. Magnesiumlegierung-Warmwalzvorrichtung nach Anspruch 3 oder 4, wobei Folgendes bereitgestellt wird:
eine Spannungsausübungsvorrichtung (8), die auf der stromabwärts gelegenen Seite der stromabwärts gelegenen Temperaturerhaltungsvorrichtung (6) angeordnet ist und eine Spannung auf die Magnesiumplatte (M1) ausübt, und
eine Aufwickelvorrichtung (7), die weiter auf der stromabwärts gelegenen Seite angeordnet ist als die Spannungsausübungsvorrichtung (8) und auf welche die Magnesiumplatte (M1) gewickelt wird.

## Revendications

1. Procédé de laminage à chaud d'un alliage de magnésium, comprenant:
une première étape de laminage dans laquelle une plaque de magnésium (M1) est laminée en un mouvement de va-et-vient entre un four à réchauffer en amont (2), qui est situé sur un côté en amont d'un laminoir (1) et qui chauffe la plaque de magnésium, et un four à réchauffer en aval (3) qui est situé sur un côté en aval du laminoir (1) et qui chauffe la plaque de magnésium (M1); **caractérisé par le fait qu'**il comprend, en outre:
une seconde étape de laminage dans laquelle la température des parties d'extrémité respectives de la plaque de magnésium (M1) sur le côté en amont et sur le côté en aval est maintenue, pendant le laminage de la plaque de magnésium (M1) en un mouvement de va-et-vient, entre un appareil de maintien de température en amont (5) qui est situé plus loin, sur le côté en amont, que le four à réchauffer en amont (2) et qui transporte la plaque de magnésium (M1) qui a été chauffée par le four à réchauffer en amont (2) tout en maintenant sa température, et un appareil de maintien de température en aval (6) qui est situé plus loin, sur le côté en aval, que le four à réchauffer en aval (3) et qui transporte la plaque de magnésium (M1) qui a été chauffée par le four à réchauffer en aval (3) tout en maintenant sa température.

2. Procédé de laminage à chaud d'un alliage de magnésium selon la revendication 1, dans lequel il est prévu une étape d'enroulement dans laquelle, tandis qu'une tension est appliquée, au moyen d'un dispositif d'application de tension (8) qui est situé sur le côté en aval de l'appareil de maintien de température en aval (6), sur la plaque de magnésium (M1) qui a été laminée à une épaisseur prédéterminée, la plaque de magnésium (M1) est enroulée sur un enrouleur (7) qui est situé plus loin, sur le côté en aval, que l'appareil de maintien de température en aval (6).

3. Dispositif de laminage à chaud d'un alliage de magnésium, comprenant:
un laminoir (1) qui effectue un laminage en va-et-vient sur une plaque de magnésium (M1);
un four à réchauffer en amont (2) qui est situé sur le côté en amont du laminoir (1) et qui chauffe la plaque de magnésium (M1); et
un four à réchauffer en aval (3) qui est situé sur le côté en aval du laminoir (1) et qui chauffe la plaque de magnésium (M1);
**caractérisé par le fait que** le dispositif comprend, en outre:
un appareil de maintien de température en amont (5) qui est situé plus loin, sur le côté en amont, que le four à réchauffer en amont (2) et qui transporte la plaque de magnésium (M1) qui a été chauffée par le four à réchauffer en amont (2), et qui maintient également la température des parties d'extrémité sur le côté en amont; et
un appareil de maintien de température en aval (6) qui est situé plus loin, sur le côté en aval, que le four à réchauffer en aval (3) et qui transporte la plaque de magnésium (M1) qui a été chauffée par le four à réchauffer en aval (3), et qui maintient également la température des parties d'extrémité sur le côté en aval.

4. Dispositif de laminage à chaud d'un alliage de magnésium selon la revendication 3, dans lequel une pluralité de groupes de rouleaux pinceurs (4) qui tiennent la plaque de magnésium (M1) en sandwich dans le sens de son épaisseur et qui règlent sa vitesse de transport sont prévus, respectivement, entre le laminoir (1) et le four à réchauffer en amont (2) et entre le laminoir (1) et le four à réchauffer en aval (3).

5. Dispositif de laminage à chaud d'un alliage de magnésium selon la revendication 4, dans lequel des rouleaux de travail du laminoir (1) et la pluralité de groupes de rouleaux pinceurs (4) qui sont situés sur les côtés en amont et en aval du laminoir (1) sont des rouleaux chauffants.

6. Dispositif de laminage à chaud d'un alliage de magnésium selon la revendication 3 ou 4, dans lequel il est prévu:
un dispositif d'application de tension (8) qui est situé sur le côté en aval de l'appareil de maintien de température en aval (6) et qui applique une tension sur la plaque de magnésium (M1); et
un enrouleur (7) qui est situé plus loin, sur le côté en aval, que le dispositif d'application de tension (8) et sur lequel la plaque de magnésium (M1) est enroulée.
